

S. I. CLAWSON.  
PROCESS OF VOLATILIZING ORES.  
APPLICATION FILED AUG. 4, 1909.

1,262,452.

Patented Apr. 9, 1918.



Inventor

Selden I. Clawson

By

Sturtevant & Mason

Attorneys

Witnesses

C. M. Lacker  
Grace P. Breerton

# UNITED STATES PATENT OFFICE.

SELDEN IRWIN CLAWSON, OF SALT LAKE CITY, UTAH.

## PROCESS OF VOLATILIZING ORES.

1,262,452.

Specification of Letters Patent.

Patented Apr. 9, 1918.

Application filed August 4, 1909. Serial No. 511,204.

*To all whom it may concern:*

Be it known that I, SELDEN I. CLAWSON, a citizen of the United States, residing at Salt Lake City, in the county of Salt Lake, 5 State of Utah, have invented certain new and useful Improvements in Processes of Volatilizing Ores, of which the following is a description, reference being had to the accompanying drawing, and to the letters and 10 figures of reference marked thereon.

The invention relates to a process of treating ores, and more especially the volatilization of roasted ores. While various ores may be treated by my process, it is more especially adapted for use in connection with the reduction of ores containing gold, silver, copper, lead, zinc, antimony or bismuth. 15

In the extraction of gold, silver, copper and lead from ores by the process of volatilization, it is necessary to heat the ore to a considerable degree. I have found that these volatile metals are much more advantageously caught after the extraction from the gangue, if the volume of air carrying 25 the metal is comparatively small.

The object of this invention, therefore, is to provide a process of extracting the metal from the ore, wherein a comparatively small amount of air carries the metal to the 30 fume arrester. I have found this can be accomplished if the fire gases used in heating the ore to the volatilization point are excluded from the fume arrester.

The invention consists in preheating or 35 roasting the ore in an oxidizing chamber not of the muffle type, wherein the fumes and gases are allowed to escape, after which it is passed in its heated state to a second chamber, where it is again heated and the 40 fumes or gases conveyed to a fume arrester. The ore may be treated with chlorin gas in the volatilizing chamber, or may be treated with a flux, as it is passed from the preheating chamber to the volatilizing chamber. 45 Or the ore may be fluxed before entering the preheating chamber, the gases and air being allowed to escape from said chamber. The transfer of the ore to the volatilization chamber occurs before the volatilization of 50 the metals takes place.

In carrying out the invention, I prefer to use the herein described apparatus, wherein two furnaces are arranged in tandem, but it will be understood that other arrangements may be used, and that other types of fur-

naces may be used from those herein described, without departing from the spirit of my invention.

The figure in the drawing shows more or less diagrammatically and in section an apparatus for carrying out the invention.

The apparatus consists of a furnace 1, which, as herein shown, is of the ordinary revolving type. The crushed ore is fed to a hopper 2, and from the hopper 2 by a screw conveyer to the furnace 1. A furnace 3 is located at one end of the furnace 1. Said furnace 3, as herein shown, consists of a closed chamber having a pipe 4 leading to a fume arrester 5, which may be of any desired type. The fire box 6 located beneath the furnace 3 serves as a means for heating the furnace, and the pipe 7 conveys the gases and fumes from the fire box to the furnace 1. 75

The ore passes through the furnace 1, and is fed into the chute 8, which leads to the furnace 3. A hopper 9 may be provided with a flux, which is fed by means of the conveyer 10 to the ore, as it passes from the furnace 1 to the furnace 3. A pipe 11 leads into the bottom of the furnace 3, and may be used to convey chlorin gas to the furnace 3. Air may be fed to the pipe 11 through the auxiliary pipe 12, if desired. 80

The ore as it passes from the furnace 1 to the furnace 3, will pile up in the furnace and close the lower end of the chute 8, so that the fumes and gases from the furnace 3 will pass through the pipe 4 to the fume 90 arrester. A suitable opening 13 may be formed in the front of the furnace 3, through which the ore in said furnace may be raked and drawn through the opening, when desired. A little air may 95 be fed to the furnace through the opening 13, whenever it is found desirable. Said opening may be closed by any suitable door.

In carrying out my improved process, the fire box 6 is charged, and the furnace 3 100 thoroughly heated. The fumes from the fire box also pass to the furnace 1, which becomes heated.

The chlorin generator for supplying the chlorin gas and the fume arrester are, of course, put into shape for operation. The crushed ore is now fed to the hopper 2, and the ore is then passed by the screw conveyer to a point inside of the furnace 1. The ore travels through the revolving fur- 110

nace 1, becoming heated more and more until the sulfurous particles in the ore take fire, after which the ore drops out of the furnace into the chute 8, and passes down into the 5 volatilization chamber or muffle 3.

The ore accumulating in the muffle or furnace 3 piles up in the chute, so that there will be no draft passing up through the chute. It will be noted that as the ore passes 10 through the furnace 1, the fumes and gases therefrom pass through the stack connected with the furnace. The ore in this furnace is heated to the chemical re-action point, or to a point a little below the point of tem- 15 perature at which the metal chlorids volatilize.

When the ore reaches the furnace 3, the chlorin gas of the flux which is mixed with the ore as it passes to the furnace, brings 20 about the desired chemical re-action, and the fumes or gases rising from the ore will pass through the pipe 4 to the fume arrester.

It will, therefore, be seen that a comparatively small amount of air containing the 25 volatile metals passes through the fume arrester, which greatly increases the efficiency thereof.

It should be understood that in carrying out my process, I do not desire to be limited 30 to any particular type of preheating or volatilization furnace. The preheating furnace might consist of a simple roasting furnace of any well known type, and, on the other hand, the volatilization furnace might 35 consist of any revolving muffled furnace or

a reverberatory furnace, or any other like kind of furnace.

The essential features of my invention consist in preheating the ore to a point a few degrees below the point of volatilization of the metals, the fumes and gases being allowed to escape during preheating, and then heating the ore to a higher temperature in a substantially closed chamber, and passing the fumes and gases which contain a 40 comparatively small amount of ore from said chamber to the fume arrester. It is understood, of course, that the ore would be crushed and rabbled, as conditions demand.

Having thus described my invention, 50 what I claim as new and desire to secure by Letters Patent, is:—

The process of treating ores by volatilization consisting in subjecting the ore directly to fire box gases for a time for pre- 55 heating the same to a temperature below that at which the metal chlorids would volatilize and allowing the fumes and gases to escape during such preheating, treating the heated ore while still hot with a halogen reagent and subsequently volatilizing the halogen compounds out of the ore and passing the products of volatilization to a fume arrester.

In testimony whereof I affix my signature, 60 in presence of two witnesses.

SELDEN IRWIN CLAWSON.

Witnesses:

W.M. T. FOULGER,  
W. J. BARNES.